

Oct. 20, 1925.

F. H. CHAPIN

1,558,237

METHOD OF MANUFACTURING SHRINK HEAD CASINGS

Filed April 20, 1925



Fred H. Chapin,  
By Hell, Brock West,  
Atlys.

Patented Oct. 20, 1925.

1,558,237

# UNITED STATES PATENT OFFICE.

FRED H. CHAPIN, OF CLEVELAND, OHIO.

## METHOD OF MANUFACTURING SHRINK-HEAD CASINGS.

Application filed April 20, 1925. Serial No. 24,684.

To all whom it may concern:

Be it known that I, FRED H. CHAPIN, a citizen of the United States, residing at Cleveland, in the county of Cuyahoga and State of Ohio, have invented a certain new and useful Improvement in Methods of Manufacturing Shrink-Head Casings, of which the following is a full, clear, and exact description, reference being had to the accompanying drawings.

This invention relates to what are known in the art of ingot casting as feeders, sink heads, hot tops, or more properly shrink-head casings for ingot molds, the function of which is to delay the cooling or solidification of the molten metal in the upper part of the solidifying ingot so that during the shrinkage of the ingot a pipe or shrinkage cavity is not formed in the major part thereof and is confined to a relatively small part of the upper portion of the ingot formed within the shrink-head casing. This function of the casing is well understood by those skilled in the art and is more fully described in my application for patent filed Apr. 20, 1925, No. 24,685, in which claims are made to the construction and composition of the casing made by the method herein described and claimed.

In the accompanying drawings Fig. 1 is a perspective view of a shrink-head casing made in accordance with my invention; and Figs. 2 to 9 inclusive indicate the various successive steps employed in the manufacture of such casings.

Ordinarily heretofore shrink-head casings have been made of refractory material such as fire clay or fire brick material which is extremely hard and brittle, having been baked at a very high temperature and having a texture which is quite close. In order to make such casings, special plants have been required; it has not been the practice to make such casings at steel plants. Thus transportation of the casings has been necessary and the expense is correspondingly increased. When in use, the fire clay or fire-brick casings have been supported on the molds by some means which allow them to descend into the mold cavity as the ingot shrinks and solidifies. This has been found necessary as the casing adheres to the top of the ingot and, unless it is allowed to lower with the shrinking ingot, it will be broken and prematurely destroyed. When the casting operation is finished, the casing remains

on top of the ingot and is usually broken up by hammers or other suitable tools and thus removed from the ingot before the latter is reheated and passed to the rolls for reducing the ingot to the desired shape. Quite frequently, lumps and finer particles of clay remain on the ingot and become embedded therein while passing through the rolls, thus making flaws in the rolled product which are sometimes serious.

Shrink-head casings made of fire clay have rather low heat-insulating qualities, necessitating the loss of a considerable quantity of metal from the top of the ingot where the pipe or cavity occurs, it being necessary to remove or crop this portion of the ingot after it and the sound portion thereof are rolled into blooms, billets, and other shapes.

It is the object of my invention to overcome the defects ordinarily found in shrink-head casings as heretofore made, and I have devised a way of making such casings of material which is not only much cheaper than fire-clay or similar refractory material, but which will produce casings of greater efficiency because possessing characteristics which entirely eliminate some of the difficulties heretofore encountered in the use of clay casings.

I have found that if blast furnace slag is properly prepared and mixed in ordinary cold water in proper proportions with commercial Portland cement, it may be molded into proper shape for use as shrink-head casings and that, if the surface of such a casing be treated with a suitable substance, it will be rendered water-proof or non-absorbent of liquids or gases. This treatment of the casing prevents the formation of such gases in the interior of the casing as would produce an endo-thermic action in connection with the molten metal contacting with the casing which would result in what is known in the art as a "boil", or such a disturbance in the forming ingot as to impede or mar the proper casting of the ingot, and the formation of gases in the casing which would crack or break it.

The particular shape of the casing, so far as the present invention is concerned, is not essential. Various shapes may be used, but that illustrated in Fig. 1 of the drawings is preferred. As shown, the casing B is generally rectangular in horizontal cross section. The lower part of the casing is rounded at the four corners, as indi-

cated at *a*, thus producing a lower part *b* which is adapted to enter the mold cavity and shoulders *c* which are adapted to rest on the top of the mold and thus support the casing.

While I prefer to mold the casing in one integral piece, it may be made in sections. When the mold is of large size, a sectional casing may be found preferable.

10 Heretofore shrink-head casings have ordinarily been made of refractory material, such as fire clay, which is baked at a high temperature at which it has been impossible to obtain casings in quantity production of uniform density or porosity, as some of the casings are invariably burnt at a higher temperature than others in the same lot or kiln; and this baking has been performed in a special plant remote from the steel plant. The casings made in accordance with my invention are made of relatively low-refractory material, baked or hardened at a relatively low temperature, and may be made at the steel plant, inasmuch as I employ furnace slag as a principal ingredient of the casing and combine such slag with a suitable proportion of commercial Portland cement, which is readily obtainable. Blast furnace slag gives the best results, although open hearth or other slag may be used.

In the manufacture of shrink-head casings according to my invention, ordinary furnace slag taken from the dump is ground or crushed by suitable machinery until it is in proper condition to be screened. The crushed or ground slag is then screened in preferably a screen of  $\frac{1}{4}$  inch mesh. In this way the larger lumps are separated from the dust and smaller particles.

The screened slag is then thoroughly mixed and blended with Portland cement in a suitable mixer and while dry. Preferably one part of the cement is mixed with seven parts of slag by weight, as these proportions are found to give the best results, although they may be varied. After being thoroughly mixed and blended, a sufficient amount of ordinary cold water may be added to the blended material while they are in the same mixer, or the blended dry cement and slag may be transferred to another container where water is added and the ingredients thoroughly kneaded and mixed until a mass of desired consistency for molding is produced. The material is then in condition to be molded and suitable molds may be used for this purpose, the material being packed in the molds and rammed or tamped in the usual way until the desired shape is obtained.

The next step in the process is to remove the free moisture from the casings, and this is done by heating the casings for about 12 hours in what is called a pre-

liminary dryer, at a temperature of from about  $200^{\circ}$  to  $250^{\circ}$  F. By this step in the process, all free moisture is eliminated from the casing and the setting of the cement is hastened. The cement acts as a binder, and I preferably use commercial Portland cement as such binder, although other materials might be used for this purpose with fairly good results. When dried and baked at the temperature specified, the casing is rendered porous and is in good condition to receive the impregnating liquid or substance which serves to render inactive the gas producing constituents of the material of which the casing is made and to thus prevent the formation and liberation of gases from the casing when the latter is subjected to the intense heat of the ingot while being formed. For this purpose I preferably employ a substance sold as "Goulac," well known to foundry men and which consists mainly of organic matter (cellulose) with the following additional ingredients:—

Aluminum oxide ( $Al_2O_3$ ).

Ferric oxide ( $Fe_2O_3$ ).

Manganese oxide ( $Mn_2O_3$ ).

Calcium oxide ( $CaO$ ).

Magnesium oxide ( $MgO$ ).

Sulphur (S).

The cellulose in the "Goulac" is that obtained from the dried liquor from the manufacture of sulphite pulp. A non-organic compound such as magnesium fluosilicate may also be used instead of "Goulac." The impregnating substance may be applied by spraying, brushing, or by dipping the casing into a bath of the liquid whereby all the walls are impregnated to a suitable distance with the impregnating substance. While good results have been obtained where the impregnation extends from  $\frac{1}{8}$  to  $\frac{3}{4}$  inch into the casing walls, it is preferable to impregnate the casings completely, as indicated by the stippling at X in Fig. 1. The impregnating material serves to render inactive the gas producing constituents of the material of which the casing is made as above stated, and also renders the casing as a whole substantially water-proof so that it will not absorb moisture and thus render the porous casing liable to rupture through the formation of steam therewithin.

After being thus treated, the casings are baked in a suitable furnace for about 12 hours, the latter being heated to a temperature of from  $600^{\circ}$  to  $800^{\circ}$  F. which, it will be observed, is not only a much lower temperature than that employed for burning fire clay, but one which will not fuse the slag ingredients of the casings. When thus baked, the casings are complete and ready for use on the molds.

The time occupied in the preheating or preliminary heating and the final heating

is readily determined, it being important in the first heating to drive off the moisture in the form of steam and in the second case to dry and harden the surface of the casing 5 where the water-proofing or impregnating substance is contained. As pointed out hereinbefore, about 12 hours will be sufficient for each of these heating operations.

While I prefer to apply the impregnating substance to the entire exterior of each casing, it may be applied only to the inner walls thereof which come in contact with the molten metal of the forming ingot, and I may apply other forms of water-proofing 15 material to other parts of the casing.

Inasmuch as the interior of each casing is porous and substantially moisture-free, it serves as a heat insulator, and the metal of the forming ingot at the top of the mold 20 is maintained in liquid condition until the formation of the ingot is completed.

As explained in my application for patent above referred to, while my casing is in use the hot molten metal which rises in it when 25 the mold is being poured softens the inner walls of the casing, due to the fusion of the slag content thereof, and renders them non-adherent to the ingot, so that as the forming ingot shrinks it will draw away from the 30 casing without imparting harmful strains thereto. The substance with which the casing is treated prevents the swelling or spawling of the slag constituent of the casing and thus enables the ingot to free itself 35 from the inner walls of the casing during the solidification and shrinkage thereof.

My invention while especially designed for use in connection with molds for forming steel ingots, may be employed in connection with molds of other kinds or molds 40 for forming other kinds of castings. While slags and refractories of various chemical compositions will produce articles having the advantages referred to, the best results 45 I have found by many experiments are obtained by using a blast furnace slag containing a substantial proportion of magnesia.

It has been stated that the plant for making the casings is conveniently located at the steel plant where the slag is found, but it is of course feasible to make the casings in plants remote from the steel plants, although this involves transportation and additional expense. In any event, by using a 50 waste product such as slag in connection with a relatively small percentage of cement or other binding material, my casings may be made very much more cheaply than can 55 those made of fire clay; and such casings made in accordance with my invention possess the beneficial characteristics set forth hereinbefore, which are not found in casings heretofore employed.

60 This application is a continuation in part

of my application No. 738,774 filed September 20, 1924 and of my application No. 758,594 filed December 29, 1924.

Having thus described my invention, what I claim is:

1. In the manufacture of shrink head casings for ingot molds, the method herein described which consists in mixing furnace slag and a binder in proportions of about 7 parts by weight of slag to one part by 75 weight of the binder, molding the mixture to give it the desired shape and then baking the molded article at a temperature of between 200° and 250° F. to remove moisture therefrom and render the casing porous. 80

2. In the manufacture of shrink head casings for ingot molds, the method herein described which consists in mixing blast furnace slag and cement in proportions of about 7 parts by weight of slag to 1 part 85 by weight of cement in water, molding the mixture to give it the desired shape, and then baking the molded article at a temperature of between 200° and 250° F. to remove moisture therefrom and render the casing 90 porous.

3. The method herein described of making shrink head casings for ingot molds which consists in mixing refractory material and a binder in water, molding this 95 mixture, removing moisture from the molded article, and then treating the casing with a substance which renders inactive the gas forming constituents contained in the casing. 100

4. The method herein described which consists in mixing refractory material and a binder in water, molding this mixture, baking the molded article to remove moisture therefrom, treating the molded article with a substance which render inactive the 105 gas forming constituents in the casing, and finally baking the casing at a relatively high temperature but below the fusing point of the contained refractory material. 110

5. The herein described method of making shrink head casings for ingot molds which consists in mixing furnace slag and cement in water, molding this mixture to give it the desired form, baking the molded article to remove moisture therefrom and to render the casing porous and absorbant, 115 treating the casing with a substance which renders inactive the gas forming constituents of the ingredients of which the casing is made, and finally baking the casing at a relatively high temperature but below the fusing point of the slag constituent thereof. 120

6. The herein described method of making shrink head casings for ingot molds which consists in mixing refractory material and a binder in water, molding the mixture to give the desired form thereto, baking the molded article at a low temperature to drive out the moisture from the casing and render it porous and absorbent, 125 130

4

applying a substance to the inner wall of the casing which serves to render inactive the gas forming constituents therein, and then baking the casing at a relatively high 5 temperature to harden it.

7. The method of manufacturing a shrink head casing for an ingot mold which consists in mixing binding material with refractory material which is fusible at the 10 temperature of the molten metal of an ingot, molding the mixture to give it the desired shape, heating the molded article thus formed to dry the same without fusion thereof, treating the metal contacting portions 15 of the casing with a substance which renders inactive the gas forming constituents in the casing and then baking the casing at a relatively high temperature but lower than the fusing point.

20 8. The method herein described of mak-

ing shrink head casings for ingot molds which consists in forming a porous moisture free casing from furnace slag and a binder, impregnating such casing with a substance which renders inactive the gas 25 forming constituents of the casing, and then baking the impregnated casing at a temperature below the fusing point of the slag.

9. In the manufacture of shrink head casings for ingot molds, the method herein 30 described which consists in molding refractory material while in a plastic condition to give it the desired shape, and in treating the refractory material from which the casing is formed with a substance which 35 renders inactive the gas forming constituent of the material.

In testimony whereof, I hereunto affix my signature.

FRED H. CHAPIN.